

## UNITED STATES PATENT OFFICE

2,190,034

METHOD OF MAKING WATERPROOF  
SHEETS OR BOARDS

Harold L. Levin, Nutley, N. J., assignor, by mesne assignments, to The Patent and Licensing Corporation, New York, N. Y., a corporation of Massachusetts

No Drawing. Application January 30, 1931,  
Serial No. 512,497

2 Claims. (Cl. 92—21)

This invention relates to improvements in the art of making waterproof sheets or boards, particularly sheets or boards having waterproof and thermo-plastic properties to render the product suitable for use in the fabrication of automobile panel board, flooring, box board, roofing elements, shoe elements, gaskets, binder board, interior or exterior facing or veneer panels, advertising signs, artistic or ornamental plaques or the like. An object of the invention is to provide an improved process for effectively combining a waterproof and/or thermo-plastic substance with fibrous pulp for the production of a stock that can be successfully run on a paper making machine for the formation of homogeneous fibrous sheets or boards carrying substantial quantities of the waterproof and thermo-plastic binder uniformly distributed therethrough.

More specifically an object of the invention is to provide a process of dispersing or disintegrating normally friable, thermo-plastic, bituminous or bitumen-pitch type substances in the presence of wet pulp which acts as a peptizing agent, to a sufficiently fine degree of subdivision or dispersion as to render the particles capable of being adsorbed on the surface of the fibres contained in the pulp.

I have found in accordance with the present invention that a binder of the character indicated may be conditioned as aforesaid by a continued mechanical impact as for example, under the action of the beater roll of an ordinary paper mill beater, in the presence of wet pulp circulating in the beater.

The process of my invention is adapted particularly for the utilization of bituminous substances of a more or less hard friable character, such as typified by asphalts having penetration and melting point relationships within a range in which they lend themselves to grinding at normal atmospheric temperatures to a state in which the particles do not coalesce but on storage undergo incipient sintering so as to adhere to each other sufficiently so that some light mechanical dis-

placement is required to restore the individualized condition; but in which range they are susceptible to fusion and coalescence at temperatures comparable to those usually prevailing on the steam heated driers of a paper making machine.

The bituminous substances especially contemplated for use in accordance with my invention, generally speaking, have a steep susceptibility curve; that is to say they are susceptible to noticeable changes in penetration with slight changes in temperature. Accordingly, my in-

vention may be considered as applicable to the use of asphalts ranging in hardness from zero penetration (at 77° F. standard method of test) and melting point of 200° F., to those having a penetration of about 15 and a melting point upwards of 135° F. to approximately 200° F.

In carrying out my invention in one of its embodiments, an ordinary paper mill beater may be charged with a suitable quantity of fibrous pulp and while the latter is being circulated therein, the desired quantity of an asphalt of the character above set forth, in the form of small lumps or chunks, may be slowly fed to the beater, while the contents thereof are maintained at normal atmospheric temperatures, say 77° F., but preferably not in excess of 100° F. At the beginning of the operation it may be necessary to raise the beater roll to some substantial distance above the bed plate in order to avoid undue mechanical strain that may be imposed by contact with the lumps or chunks of relatively hard asphalt circulating in the beater. As the action of the beater is continued or prolonged the lumps or chunks of asphalt will gradually become reduced to smaller fragments, as a result of the continued impact action, and the beater roll may then be gradually lowered closer towards the bed plate so that on continued action the size of the asphalt particles will be progressively reduced. The operation is thus carried on until the asphalt is reduced to particles of very small size which for the purposes of my invention should approximate an average particle size of about 35 mu. This serves to bring about a condition in which the particles of the asphalt have developed sufficient surface energy so that they are capable of being adsorbed on the surface of the fibres contained in the stock and carry minute electric charges giving them capacity for ion adsorption and ability to respond to the action of flocculating electrolytes. I consider this to be a rather important or significant feature of my invention, as it insures the attainment of numerous advantages of the invention as herein set forth and also serves as a guide in controlling the operation. In this latter respect it may be here pointed out that as the asphalt becomes disintegrated under the action of the beater into fragments of small size the color of the stock, as for example the grayish color that typifies news stock, will gradually change to the color of the asphalt, the gradation in the color becoming more apparent as more asphalt is put in and as the asphalt becomes more finely divided, until when the particles have been reduced to a size approxi-

mating that indicated, only substantially small proportions of the asphalt particles will be discernible by the eye as discrete particles separate from the fibre and the stock takes on a homogeneous condition uniformly of the color of the asphalt. This condition will therefore serve as a guide to the operator as indicating the sufficiency of the subdivision of the asphalt and ensures a condition which contributes greatly to the 10 operation without gumming the instrumentalities of the paper machine, wet or dry end, and ensures uniform coating of the fibres when the product has been coalesced in the drying action.

The quantity of asphalt that may thus be combined advantageously with fibrous pulp may vary up to several times the weight of the fibre in the stock and the exact quantity employed may accordingly be governed largely by the degree of 15 waterproofness and/or thermo-plasticity desired 20 in the product.

An important advantage of the operation thus described resides in the fact that it avoids the necessity for employing special equipment for 25 conditioning the asphalt since the entire operation 30 may be effectively carried on in an ordinary paper mill beater.

In respect to the advantages accruing from the process of my invention, according to which the asphalt may, and preferably is, caused to be 35 subdivided into particles approximating the size hereinabove specified, I have found as above stated, that the particles in this state of subdivision acquire electrostatic charges, and are susceptible to adsorption of ions and/or protective colloids, 40 and hence upon the addition of suitable flocculating electrolytes the pH of the system may readily be brought to the isoelectric point so as to cause the particles of asphalt to cluster, clot or deposit upon the fibres.

One of the advantages of this type of reduction 45 resides in the fact that reduction in the presence of water only, does not result in particles of the desired average degree of fineness within a reasonable time and further, when reduced with water the particles do not wet readily with water, and tend to float on the water medium.

Illustrating the application of my invention to 50 various types of fibrous stock and various bituminous substances falling within the range to which the invention is particularly applicable, I may cite as an example the use of an asphalt 55 known in the trade as B-grade California, having a penetration of 4 at 77° F. and a melting point of 175° F. which may be worked up in the manner hereinabove described with a fibre furnish consisting substantially entirely of news, in the proportion of approximately equal parts of dry fibre and asphalt. A selected grade of coal tar pitch corresponding in properties approximately to the 60 B-grade California asphalt may similarly be employed.

Another example of ingredients that may be employed in carrying out the invention, particularly for the production of a light colored sheet 65 or board is illustrated by the use of an asphalt known in the trade as Albino asphalt which is an asphalt characterized by a low asphaltene content and derived from a Borneo crude, and having a penetration of approximately 12 and a melting 70 point of approximately 135° F. This may be worked up with an equal part by weight of a fibre furnish consisting approximately of equal parts of news and kraft. Inasmuch as asphalt of this type is normally of relatively light color, suitable 75 proportions say 10 to 20% of pigment may be

incorporated in the stock where a colored product is desired. Thus the furnish may be as follows:

|                   | Percent |
|-------------------|---------|
| Albino asphalt    | 35      |
| Red oxide pigment | 15      |
| Fibre             | 50      |

Where the fibre furnish consists entirely or largely of fibres of a character such that excessive beating may produce a stock that is not as "free" as may be desired under the condition of operation, the operation may be conducted by conditioning the bituminous material in the presence of part of the fibre furnish, in order to avoid undue shortening of the fibres and excessive hydration of the entire fibre furnish. After all of the asphalt has been dispersed the remainder of the fibre furnish may be added. Thus, for example, 300 parts by weight of an asphalt of 10 penetration and a melting point of 145° F. may be treated in the beater as above described with 100 parts by weight of kraft fibre circulating in the beater and after all the asphalt has been dispersed to the condition above described, 100 to 500 parts by weight more of kraft fibre may be added to the beater and the operation of the beater continued until the freshly added fibre has been uniformly disseminated through the stock.

In those cases where the asphalt is of a softer or less friable variety falling within the range herein specified, it may be desirable in certain instances to introduce finely divided mineral matter into the asphalt in molten condition in order to render the asphalt more readily susceptible to disintegration by the operation of my process into particles of a size approximating 35 mu. For this purpose clay, diatomaceous earth, fuller's earth, slate dust, bentonite or similar substances may be employed in quantities ranging from 20 to 50% by weight of the asphalt. Where a material such as bentonite is employed for this purpose the swelling action of the bentonite upon coming into contact with water will serve to facilitate the reduction of the asphalt to finely divided particles and in this case, as also in the case of other substances that may be employed for the purpose of rendering the asphalt more friable and susceptible to ready disintegration, the mineral matter may become adsorbed on the surface of the asphalt particles when they are reduced to the finely divided size herein contemplated, and thus serve further to stabilize the stock.

I have hereinabove referred to the ability of the asphalt particles when reduced to an average size approximating 35 mu to adsorb ions and protective colloids. Hence, where it is desired to provide additional peptization protection in the stock, substances such as bentonite, clay, animal or vegetable glue may be added to the stock in proportions of say 2 to 10% based on the dry weight. For this purpose also there may be used certain types of sulphonic acids preferably those of high molecular weight characterized by complete solubility in water and also solubility in solutions of calcium chloride. These sulphonic acids may be obtained from the acid tars resulting from the latter stages of a multi-stage sulphonation treatment of mineral oil fractions particularly lubricating oil. They may also be obtained from the acid tars resulting from the sulphonation of non-aromatic hydrocarbons insoluble in liquid sulphur dioxide.

Where it is deemed necessary or desirable to ensure complete deposition or clustering of the asphalt particles upon the fibres contained in

the stock, suitable quantities of alum or similar substances may be added, preferably, in quantities which will be sufficient to bring the pH of the stock to the isoelectric point of the colloidal system.

5 While I have heretofore specified that the selected asphalt may be added in the form of lumps or chunks to the fibrous pulp circulating in the beater, it may be desirable in some instances 10 to feed the same asphalt to the beater in a molten or heat liquefied condition thus facilitating the conveyance of the asphalt from the source of supply to the beater. It is to be understood therefore that the invention contemplates as an alternative method of introducing the asphalt into the beater, the feeding of the asphalt in molten condition. By maintaining the contents of the beater cold, substantially the same character of 15 stock may be produced with the given asphalt, as 20 where the asphalt is added to the beater in solid lumps or chunks, with all the attendant advantages thereof. In operating the process with this alternative mode of feeding the asphalt to the beater, the asphalt being at a temperature 25 above the boiling point of water, and the contents of the beater being preferably not in excess of 77° F., the expansive forces of the steam generated when the hot asphalt impinges upon the aqueous fibrous suspension circulating in the 30 beater will cause local foaming of the contents thus facilitating the reduction of the asphalt into particles of the desired size.

When the stock containing the desired types 35 and relative quantities of fibre and binder has been conditioned as above described, it may then be conducted in the usual way to and over the paper making machine for formation into sheets. Thus, the stock may be fed to one or more of the 40 cylinders of a multi-cylinder machine for the production of a multi-ply sheet and the formation dried in the usual way, the temperature of the steam heated driers being sufficient to cause the

asphalt to fuse and coalesce, with the result that a homogeneous and uniform sheet is obtained in which the asphalt is contained in substantially continuous films on the fibres. Where boards of high caliper are desired the treated stock may be 5 formed on the cylinder of a wet machine and the formation transferred by the usual blankets to the make-up roll, from which it may be stripped when the desired caliper has been built up, and dried and calendered in the usual way, thereby 10 effecting fusion and coalescence of the asphalt particles distributed therethrough on the fibres, as already described.

The various stocks prepared as above described 15 may also be formed on suction molds to form articles of hollow or irregular contour, such as fibre buckets, waste paper or other receptacles, toys, etc.

The expression "friable" as employed in the 20 claims to qualify bituminous substances generally, or asphalt specifically, is intended to embrace such materials of this type, as fall within the range of hardness herein set forth and/or are susceptible to the treatments herein described.

I claim as my invention:

1. A process of producing a dispersion of thermoplastic binder substance which comprises mixing with said binder a quantity of absorbent, finely divided non-fibrous matter under conditions to cause said binder to be absorbed by 30 said matter and form therewith a friable composition, and afterward dispersing in water the composition so formed.

2. A process of producing a pulp containing a 35 binder substance, which comprises mixing a heat plastic binder with an absorbent, finely-divided inorganic matter to the extent of producing a friable mass, disintegrating said mass, and dispersing the disintegrated mass in a pulp of fibers in water suspension.

40 HAROLD L. LEVIN.